

# UNITED STATES PATENT OFFICE.

SAMUEL MANSFIELD JONES, OF NORTH ADAMS, MASSACHUSETTS, ASSIGNOR TO  
ARNOLD PRINT WORKS, OF NORTH ADAMS, MASSACHUSETTS, A CORPORATION  
OF MASSACHUSETTS.

## MERCERIZATION.

1,346,802.

Specification of Letters Patent. Patented July 13, 1920.

No Drawing.

Application filed May 12, 1920. Serial No. 380,889.

To all whom it may concern:

Be it known that I, SAMUEL MANSFIELD JONES, a citizen of the United States, and a resident of North Adams, in the county of 5 Berkshire and State of Massachusetts, have invented new and useful Improvements in Mercerization, of which the following is a description.

This invention particularly relates to a 10 method of mercerizing cellulosic fibers of natural growth such as cotton or linen, when interwoven or intermingled with filaments of artificial silk known as viscose, while at the same time protecting such viscose filaments from deleterious attack by the caustic 15 alkali employed for mercerization.

Letters Patent No. 1,316,958, were granted to me September 23, 1919, for an invention which accomplished by its own particular 20 method therein set forth the novel utility just specified; but I have discovered that other methods are available for accomplishing the like ultimate result, and that among these is the method herein described which 25 involves the modification of the caustic alkali solution used for mercerization by introducing into it glycerin otherwise known in chemical nomenclature as glycerol.

For the purpose of the present invention 30 I find it practically satisfactory to compose the mercerizing liquid by adding glycerin in the proportion of 135 grams to 865 grams of an aqueous solution of sodium hydrate at 65° Twaddell. This proportion is not 35 rigid; but if the ratio of the quantity of glycerin to that of the caustic alkali in solution at the hydrometric density stated is much less than the ratio just indicated the viscose silk will not be adequately protected. 40 and if such ratio is much greater the mercerizing efficiency of the caustic alkali thus modified will tend to become impaired.

Otherwise than such required modification of the mercerizing solution the treatment 45 of the fabric into which mercerizable cellulosic fibers such as cotton or linen have been interwoven with viscose-silk filaments is substantially the same as that customarily employed in the mercerization of woven fabrics composed entirely of cotton including 50 the usual means and mode of applying tension thereto for the prevention of shrinkage.

The employment of a mercerizing solution of caustic alkali which has been modified

by the addition thereto of glycerin as hereinabove provided, enables the process of mercerization to be successfully practised upon cellulosic fibers of natural growth such as cotton or linen, while at the same time the viscose silk filaments interwoven with these are effectively protected against injury from the caustic alkali; so that the resulting product is expeditiously obtained without incurring the extra expense and labor required for separately mercerizing the 60 cellulosic fibers in the yarn before interweaving the same with the viscose silk.

Manifestly also this invention although especially well adapted for the production of woven mixed goods of the kind hereinabove referred to, may likewise be practised upon yarns or other unwoven textile fabrics which are composed partly of mercerizable cellulosic fibers such as cotton or linen and partly of viscose-silk filaments and which are subjected to any well-known and acceptable process of mercerization suitable for imparting luster to the cellulose components of a fabric thus constituted; except only that instead of employing therein the old 80 mercerizing chemical agent alone there is to be substituted therefor a solution of caustic alkali modified by the addition of glycerin, whereby injury to the viscose components of the fabric is avoided.

I claim:

1. The method of treating textile fabrics composed of mercerizable cellulosic fibers intermixed with artificial silk filaments of viscose, for the purpose of mercerizing such 90 cellulosic fibers without injury to the viscose silk, by subjecting the composite fabric thus constituted to a process of mercerization wherein the solution of caustic alkali is modified by the addition thereto of glycerin.

2. The method of treating textile fabrics composed of yarn spun from mercerizable cellulosic fibers and interwoven with artificial silk filaments of viscose for the purpose 100 of mercerizing the fibers of such yarn without injury to the viscose silk, by subjecting the woven fabric thus constituted to a process of mercerization wherein the solution of caustic alkali is modified by the addition 105 thereto of glycerin.

3. The method of treating textile fabrics composed of cotton fibers intermixed with

artificial silk filaments of viscose, for the purpose of mercerizing such cotton fibers without injury to the viscose silk, by subjecting the composite fabric thus constituted, to a process of mercerization wherein the solution of caustic alkali is modified by the addition thereto of glycerin.

4. The method of treating textile fabrics composed of cotton yarn interwoven with

artificial silk filaments of viscose for the purpose of mercerizing the fibers of such cotton yarn without injury to the viscose silk, by subjecting the woven fabric thus constituted to a process of mercerization wherein the solution of caustic alkali is modified by the addition thereto of glycerin.

SAMUEL MANSFIELD JONES.